

Patented Sept. 15, 1953

2,652,331

# UNITED STATES PATENT OFFICE

2,652,331

## 4-AMINO-N,N-DIALKYL-3-DIALKYLAMINO-ANILINES AS DEVELOPERS FOR PHOTOGRAPHIC SILVER HALIDE EMULSIONS

Arnold Weissberger and John R. Thirle, Rochester, N. Y., assignors to Eastman Kodak Company, Rochester, N. Y., a corporation of New Jersey

No Drawing. Application December 15, 1951,  
Serial No. 261,912

10 Claims. (Cl. 95—88)

1

This invention relates to developing agents and developer compositions of use in photography and of particular use in color photography.

Primary aromatic amino silver halide developing agents, such as the p-phenylenediamines, are well known. The simpler developing agents of this type have characteristically low development rates for silver halide compared to other developing agents such as the aminophenols, and efforts have been made to increase the development rate by substitution of the aromatic nucleus or an amino group of the phenylene diamines. When the developing agents are to be used for forming dye images in color photography it has been desirable that such increases in development rate, obtained by substitution of the parent compounds, should not be accompanied by changes in light-absorption characteristics or color of the dye image obtained therefrom by coupling with a given coupler compound.

We have discovered a class of substituted p-phenylenediamine developing agents which surpass the large proportion of p-phenylenediamines in developer activity. In addition, when these developing agents are used in color-development processes of color photography, these developing agents possess very high coupling efficiencies with well known coupler compounds to yield dye images without undesirable variations in light absorption characteristics.

The developing agents of the invention have the following general structure:



wherein R and R<sub>1</sub> represent alkyl groups preferably containing from 1 to 4 carbon atoms in the carbon chain, e. g. methyl, ethyl, propyl, isopropyl and butyl groups. Of the many p-phenylenediamines investigated, only a few compounds e. g. 3,4-diamino-N,N-diethylaniline, exhibit higher development rates than our compounds, yet our compounds possess similar high coupling capacities in color photography. The compounds of the invention are similar in structure to the 3-monoalkylamino-4-amino-N,N-dialkylanilines but in contrast to such developing agents, our compounds, particularly the 3-dimethylamino-4-amino-N,N-dialkylanilines, show little or no tendency toward the mentioned variations in light absorption characteristics. That is, the former compounds having the 3-monoalkyl amino group, produce phenazonium dye images with coupler compounds, and our com-

15 pounds produce azomethine dye images. Thus with a given coupler compound no substantial variations in light absorption are obtained when the 4-amino-N,N-dialkylanilines are substituted in the 3-position with dialkylamino groups according to our invention to increase their development rates and coupling efficiencies.

Representative 3-dialkylamino-4-amino-N,N-dialkylaniline compounds of the invention are prepared as follows:

Example 1.—4-amino-N,N-diethyl-3-dimethylaminoaniline sulfate N,N-diethyl-3,4-dinitroaniline.



20 To 3 kg. of concentrated sulfuric acid at —20 to 0° is added with stirring 149 g. (1 mole) of diethylaniline. A nitration mixture of 153 g. of fuming nitric acid (sp. gr. 1.48) in 500 cc. of concentrated sulfuric acid is then added over a period of 1 1/4 hours, keeping the temperature at —8 to —10° C.

25 The mixture is stirred for 2 hours longer, then poured onto 7 kg. of ice. After standing overnight, the mixture is filtered and the orange crystals washed until neutral to litmus. Two crystallizations from ethyl alcohol, the first in the presence of decolorizing charcoal, give 61.0 g. (25.6%), M.P. 94—50.

30 *N,N-diethyl-3-dimethylamino-4-nitroaniline*.—A mixture of 15.0 g. (0.077 mole) of N,N-diethyl-3,4-dinitroaniline, 30 cc. of 25% aqueous dimethylamine and 150 cc. of 95% ethanol was heated for three days in a pressure bottle at 100°. The reaction mixture was concentrated and chilled in ice, giving 13.8 g. (92%) of orange crystals, M.P. 63.5—64.5°.

35 *4-amino-N,N-diethyl-3-dimethylaminoaniline sulfate hydrate*.—A mixture of 7.1 g. (0.03 mole) of N,N-diethyl-3-dimethylamino-4-nitroaniline and a liberal amount of Raney nickel catalyst in 60 cc. of absolute alcohol was shaken under 40 p. s. l. of hydrogen without heating. When reduction was complete, the catalyst was removed by filtration and the filtrate treated with 1.7 cc. (0.03 mole) of concentrated sulfuric acid in 10 cc. of 95% ethanol and 2 cc. of water. The salt 45 was precipitated as a gum by addition of ether. After three days at 0° the solid was collected and slurried with absolute alcohol. The white powder was collected and dried in a vacuum desiccator over sulfuric acid. The yield was 6.6 g. (68%), M.P. 107—109° C.

## 3

Example 2.—4-amino-*N,N*-dimethyl-3-dimethylaminoaniline sulfate *N,N*-dimethyl-3-4-dinitroaniline



To 100 g. (0.6 mole) of 3-nitrodimethylaniline in a 2 l. Erlenmeyer flask is added all at once 400 cc. of about 20% nitric acid at 20–25°. The flask is rotated slightly until all of the nitro compound is dissolved. Then 600 cc. more of 20% nitric acid is added and, after mixing, the reaction is allowed to proceed for 1½ to 4 hours, preferably 1½ hours. The reaction mixture is diluted with 1 l. of cold water and the crystals are collected on an 18-cm. Buchner funnel and washed with two 500-cc. portions of cold water, which may be followed by careful washing with cold acetone to remove polynitro compounds. The damp product is heated with 500 cc. of acetone for ½ hour at reflux and the mixture is cooled at 0–5° for ½ hour. The orange crystals are collected on a Buchner funnel and washed carefully with 250 cc. of ice-cold acetone. The yield is 57–61 g.; M. P. 177–178°.

Dilution of the acetone filtrate with 500 cc. of water, chilling, collecting the precipitate, and recrystallizing from about 75 cc. of acetone gives 6.3–7.1 g. more product, melting at 177–178°. The total yield is 63.3–68.1 g. (50–53.6%).

*N,N*-dimethyl-3-dimethylamino-4-nitroaniline



A mixture of 10.6 g. (0.05 mole) of *N,N*-dimethyl-3,4-dinitroaniline, 20 g. (0.44 mole) of dimethylamine, and 25 cc. of absolute ethanol was heated in a sealed tube at 135° for 7 hours. The tube was cooled to room temperature and opened. The contents of the tube were chilled at 0° for ½ hour, following which the red crystals were collected and dried. The yield was 8.6 g. (82.3%), M. P. 79–80.5°. Dilution of the filtrate gave 1.4 g. more of satisfactory material, making the total yield 10.0 g. (95.6%).

4-amino-*N,N*-dimethyl-3-dimethylaminoaniline sulfate hydrate



## 4

A mixture of 4.2 g. (0.02 mole) of *N,N*-dimethyl-3-dimethylamino-4-nitroaniline and a liberal amount of Raney nickel in 50 cc. of absolute ethanol was warmed and shaken for 15 minutes under hydrogen at 45 p. s. i. The filtrate was treated immediately with 1.11 cc. (0.02 mole) of concentrated sulfuric acid in 10 cc. of 95% ethanol and 2 cc. of water. The salt crystallized on standing at 0° for two days. The crystals were collected on a Buchner funnel, washed with absolute alcohol, and dried in a vacuum desiccator over Drierite. The yield was 4.4 g. (72%).

Example 3.—4-amino-*N,N*-dimethyl-3-diethylaminoaniline

2,4-dichloronitrobenzene is first prepared as follows by the method of Roberts and Turner, J. Chem. Soc. 127, 2004 (1925):



In a 500 cc. three-neck flask 190 cc. fuming nitric acid (density 1.51) (450% theory) is vigorously stirred and kept at 20–25° by a running tap water bath during the gradual addition of 114 cc. m-dichlorobenzene (one hour). The clear red solution is transferred to a steam bath; heated to 65–70°, kept there for ten minutes, and poured with manual stirring into a mixture of 1500 g. cracked ice and 1000 cc. water. The gummy yellowish solid is collected by suction filtration, washed with water until free of acid, dissolved in 500 cc. methanol. The cloudy solution is filtered by suction and cooled to 0° by the addition of Dry Ice. The product is collected by suction filtration and dried in air; the faintly yellow needles weigh 93 g. (48% theory) and melt at 30–31°.

5-chloro-*N,N*-diethyl-2-nitroaniline is then prepared by a method similar to that of Hollerman and de Mooy, Rec. trav. chim., 35, 30 (1916) as follows:



In a 500 cc. round-bottom flask 19.2 g. 2,4-dichloronitrobenzene, 200 cc. diethylamine, and a solution of 5.5 g. anhydrous sodium carbonate in 70 cc. water are heated under reflux on the steam bath for 24 hours. Sodium chloride is removed by filtration; the filtrate is allowed to evaporate (in a hood) to a brown oil which is dissolved in 300 cc. diethyl ether. The ether solution is washed with 100 cc. water which is then extracted with 100 cc. ether. The combined ether phases are dried over sodium hydroxide, filtered, and distilled. A clear, light red oil is collected at 93–98°/2 mm. weighing 12.5 g. which is dissolved in 25 cc. methanol. The solution is cooled by the addition of Dry Ice to –10°, filtered by suction. The product is washed with

cold methanol and dried over sulfuric acid under reduced pressure. An orange-yellow crystalline powder is obtained weighing 10.7 g. (49% theory) and melting at 30-31°.

| Analysis                              | C    | H   | Cl   | N    |
|---------------------------------------|------|-----|------|------|
| Calculated for $C_{10}H_{13}ClN_2O_2$ | 52.5 | 5.7 | 15.5 | 12.2 |
| Found                                 | 52.6 | 5.7 | 15.5 | 11.8 |

**5** **N,N-dimethyl-3-diethylamino-4-nitroaniline** is prepared by heating a mixture of 0.1 mole of the 5-chloro compound prepared above, 0.5 mole of anhydrous dimethylamine and 25 cc. of absolute alcohol in a sealed tube at 120° C. for 8 days. The solution is then diluted carefully with water and the crystals obtained from a non-polar solvent. The resultant product is then hydrogenated over Raney nickel catalyst and treated with sulfuric acid as described in the preceding examples to obtain the desired product, 4-amino-3-diethylamino-N,N-dimethylaniline sulfate.

**Example 4.—4 - amino - N,N-diethyl-3-diethylaminoaniline**

**20** A mixture of 0.1 mole of 5-chloro-N,N-diethyl-2-nitroaniline and 0.5 mol of anhydrous diethylamine and 25 cc. of alcohol are heated as above in a sealed tube to obtain N,N-diethyl-3-diethylamino-4-nitroaniline. After purification of the product by recrystallization it is reduced as in the above examples to obtain the desired product 4-amino - N,N - diethyl-3-diethylaminoaniline.

**25** The homologous 4-amino-N,N-diethyl-3-diethylaminoanilines contemplated by our invention are prepared in the manner of the above examples, preferably by the methods of Examples 3 and 4.

**30** When used for the formation of colored photographic images, the developers of our invention may be used in conjunction with any well-known coupler compounds such as those described in Fischer U. S. Patent 1,102,028, June 30, 1914; Mannes and Godowsky U. S. Patent 2,108,602, February 15, 1938; Mannes, Godowsky and Peterson U. S. Patent 2,115,394, April 26, 1938; and Mannes, Godowsky and Peterson U. S. Patent 2,126,337, August 9, 1938.

**35** The following examples, which are illustrative only, indicate developing solutions which may be used according to our invention.

**40** A. 3 g. 4-amino-3-dimethylamino - N,N-diethylaniline sulfate; 0.5 g. sodium sulfite; 20 g. sodium carbonate; 1000 cc. water.

B. 2 g. 2-cyanoacetylcoumarone; 2.5 cc. 10% sodium hydroxide; 50 cc. ethanol.

B is added to A.

When it is desired to use the developing agents of the invention for development of black and white images in ordinary emulsions, or for development of colored images in emulsion layers containing color forming coupler compounds only composition A above may be used. The other developing agents contemplated by our invention are used similarly for formation of silver or dye images in emulsion layers.

The developing agents described in the present invention may be used to form photographic images by development of exposed silver halide contained in the usual gelatin carrier or in carriers such as collodion, water-permeable cellulose ester or synthetic resin.

What we claim is:

1. A developing solution for producing colored

photographic images comprising as a silver halide developing agent, a compound having the general formula



**15** wherein R and R<sub>1</sub> each represent alkyl groups containing from 1 to 4 carbon atoms, and a compound which couples with the oxidation product of said developing agent at the primary amino group to form a colored image on development.

**20** 2. A developing solution for producing colored photographic images comprising 4-amino-N,N-dimethyl - 3 - dimethylaminoaniline as a silver halide developing agent, and a compound which couples with the oxidation product of said developing agent at the primary amino group to form a colored image on development.

**25** 3. A developing solution for producing colored photographic images comprising 4-amino-N,N-dimethyl-3-diethylaminoaniline as a silver halide developing agent, and a compound which couples with the oxidation product of said developing agent at the primary amino group to form a colored image on development.

**30** 4. A developing solution for producing colored photographic images comprising 4-amino-N,N-dimethyl-3-diethylaminoaniline as a silver halide developing agent, and a compound which couples with the oxidation product of said developing agent at the primary amino group to form a colored image on development.

**35** 5. A developing solution for producing colored photographic images comprising 4-amino-N,N-diethyl-3-diethylaminoaniline as a silver halide developing agent, and a compound which couples with the oxidation product of said developing agent at the primary amino group to form a colored image on development.

**40** 6. A method of developing a silver halide emulsion which comprises treating an exposed silver halide emulsion containing a latent image, with a solution containing a compound having the general formula



**45** wherein R and R<sub>1</sub> each represent alkyl groups containing from 1 to 4 carbon atoms for a sufficient time to develop the latent image to a silver image.

**50** 7. A method of developing a silver halide emulsion which comprises treating an exposed silver halide emulsion containing a latent image, with a solution containing 4-amino-N,N-dimethyl-3-diethylaminoaniline for a sufficient time to develop the latent image to a silver image.

**55** 8. A method of developing a silver halide emulsion which comprises treating an exposed silver halide emulsion containing a latent image, with a solution containing 4-amino-N,N-diethyl-3-diethylaminoaniline for a sufficient time to develop the latent image to a silver image.

9. A method of developing a silver halide emulsion which comprises treating an exposed silver halide emulsion containing a latent image, with a solution containing 4-amino-N,N-dimethyl-3-diethylaminoaniline for a sufficient time to develop the latent image to a silver image.

10. A method of developing a silver halide emulsion which comprises treating an exposed silver halide emulsion containing a latent image, 10

with a solution containing 4-amino-N,N-diethyl-3-diethylaminoaniline for a sufficient time to develop the latent image to a silver image.

ARNOLD WEISSBERGER.  
JOHN R. THIRLE.

## References Cited in the file of this patent

Beilstein "Handbuch der Org. Chem.", vol. XIII, 4th ed. (1930), p. 295.